

March 5, 1957

E. E. TALLIS ET AL

2,784,107

PRODUCTION OF ARTIFICIAL FILAMENTS, THREADS AND THE LIKE

Filed Nov. 12, 1952



FIG.1.



FIG.2.



FIG.3.



FIG.4.



FIG.5.



FIG.6.

*Inventors*

*Ernest Edward Tallis*

*John Harold Edwards*

*By their attorneys*

*Howson and Howson*

1

2,784,107

PRODUCTION OF ARTIFICIAL FILAMENTS,  
THREADS AND THE LIKE

Ernest Edward Tallis and John Harold Edwards, Coventry, England, assignors to Courtaulds Limited, London, England, a British Company

Application November 12, 1952, Serial No. 319,956

Claims priority, application Great Britain  
December 13, 1951

7 Claims. (Cl. 106—165)

This invention relates to the production of artificial filaments, threads, fibres and the like hereinafter referred to as filaments, from viscose.

It is known that viscose filaments produced by the normal spinning processes have a crenulated surface and a structure which consists of a skin and a core. The presence of the skin and core can be demonstrated by staining a cross-section cut from the filaments under specific conditions; such methods are described in the Textile Research Journal 1945, page 443. Another method of differentiating between the skin and core is by measuring the rate of axial diffusion of dyestuffs as described in Textile Research Journal 1948, page 9. In addition to the difference in dyeing affinity and in swelling property between the skin and core the cellulose molecules of the skin are believed to be more highly orientated than those of the core and for this reason it is thought that the strength of viscose fibres resides mainly in the skin. It is well-known, for example, that industrial viscose yarns such as are used in the manufacture of tyres have a much thicker skin than the normal textile fibres. Processes have been described in United States patent specifications Nos. 2,536,014, 2,535,045 and 2,535,044 for obtaining modified viscose filaments having a non-crenulated surface and a more diffuse boundary between the skin and core than unmodified filaments by spinning viscose in the presence of specific water-soluble quaternary ammonium compounds, or specific bath-soluble monoamines or specific aliphatic monoamines.

The object of the present invention is to provide a further process for obtaining modified viscose filaments.

According to the present invention a process for the production of artificial filaments, threads, fibres and the like comprises extruding viscose into a coagulating bath containing sulphuric acid and zinc sulphate wherein the spinning is carried out in the presence of more than  $\frac{1}{4}$  of a millimole and less than 5 millimoles per 100 grams of viscose of a polyalkylene polyamine having at least 3 amino groups which are not directly united to each other and which are primary or secondary amino groups.

In the drawing, Figures 1 to 6 are tracings of photomicrographs of yarn treated in different ways. Figure 1 shows a cross-section of unmodified yarn. Figure 2 shows yarn into which a polyalkylene polyamine has been introduced in accordance with the invention. Figures 3 to 6 show yarns into which different amounts of a polyalkylene polyamine have been introduced, and demonstrate the effect of varying the quantity of the polyalkylene polyamine.

In the preferred process according to the invention the polyalkylene polyamine is added to the viscose but if desired the polyalkylene polyamine can be added to the coagulating bath or to both the viscose and the coagulating bath. The preferred minimum concentration for addition to the viscose is 1 millimole per 100 grams of viscose. The filaments obtained have a much thicker skin, and the boundary between the skin and core is more diffuse

2

than those of filaments obtained under similar conditions but without the addition of the polyalkylene polyamines. By a suitable choice of the concentration of the polyalkylene polyamine the core can be practically eliminated.

5 The cross-sectional shape of the filaments is affected by the use of these polyalkylene polyamines, for example filaments having a bean shape or "dog-bone" shape can be obtained. The crenulations normally found in viscose rayon filament cross-sections are absent and the filaments obtained have a smooth surface. When axial diffusion tests are carried out on filaments of the present invention little or no penetration of the dyestuff occurs. It may be necessary, for any particular polyalkylene polyamine to carry out tests to determine the exact concentration required to give the effects desired.

The viscose preferably has a salt figure of at least 4. The coagulating bath may be of any desirable concentration, it may contain sulphuric acid, sodium sulphate and zinc sulphate, and the zinc sulphate concentration is preferably between 0.5 percent and 15 percent. The actual concentration of zinc sulphate used will depend on the type of yarn being spun. Other substances may be added to the spinning bath, such as ammonium sulphate, magnesium sulphate and glucose.

20 Examples of suitable polyalkylene polyamines which may be used to carry out the process of the present invention are diethylene triamine



30 triethylene tetramine



tetraethylene pentamine



35 pentaethylene hexamine  $\text{NH}_2\text{CH}_2\text{CH}_2(\text{NHCH}_2\text{CH}_2)_4\text{NH}_2$  and other members of the series



40 and compounds obtained by further alkylation of these polyalkylene polyamines obtained by condensing them with aliphatic alkylating agents containing more than one alkylating group in the molecule for example 1,3-dichlorhydrin, dichlorethylene and trimethylene bromide, for instance the condensation product of four moles of triethylene tetramine with three moles of 1,3-dichlorhydrin.

45 In addition to the non-crenulated surface and the increased thickness of skin with its more diffuse boundary with the core, the filaments of the present invention have 50 a lower water imbibition which is of considerable advantage for textile applications. The filaments of the present invention are more resistant to soiling and have an improved resistance to laundering and mechanical damage when wet.

55 When carrying out the process of the present invention the effect of the polyamines in the spinning can be demonstrated by adding a suitable indicator to the viscose and by measuring the distance from the jet at which the filaments become neutral. The actual distance depends 60 primarily upon the alkalinity of the viscose, the spinning speed, the spinning bath acidity, the spinning bath temperature and the filament denier. In the presence of a polyamine the neutral point is much further from the jet than is the case when the spinning is carried out under identical conditions but in the absence of a polyamine.

65 The process of the present invention enables unripened or so-called "green" viscoses to be spun. When spinning according to the process of this invention the concentration of cellulose in the freshly spun rayon filaments is appreciably increased.

70 The advantages of the process are realized to the greatest extent when it is used in conjunction with the

so-called "hot stretch" process in which the freshly spun filaments are subjected to stretching while it is passing through a bath of hot dilute acid as described in United States patent specification No. 2,192,074.

When filaments are made by the combination of the hot stretch process and the process of the present invention for use in the manufacture of composite rubber rayon articles, for example, tyres, the cords made from the filaments are of improved quality and have a greater fatigue life than similar cords produced without the process of the present invention.

The invention is illustrated by the following examples in which the percentages are by weight.

#### Example 1

A viscose was prepared to contain 7.5 percent of cellulose and 6.5 percent of caustic soda, using 37 percent of carbon disulphide on the weight of  $\alpha$ -cellulose. The viscose was cooled to 5° centigrade and 1 millimole of diethylene triamine per 100 grams of viscose were mixed in and the viscose filtered and de-aerated. When the salt figure had fallen to 6.0 the viscose was spun through a jet having 750 holes each 0.003" in diameter into a coagulating bath containing 9.5 percent of sulphuric acid, 4.0 percent of zinc sulphate and 20 percent of sodium sulphate at 48° centigrade. The length of immersion in the coagulating bath was 18 inches and it was withdrawn from the bath on to a godet at a rate of 48 metres per minute. The filaments were then stretched 65 percent between the first and second godets while they were passed through a hot stretch bath at 95° centigrade and 70 inches long. The hot stretch liquor was made by diluting spinning bath to three times its volume. The yarn, of 1650 denier 750 filaments, was subsequently washed, desulphurized, a finish was applied and the yarn was dried and collected on bobbins by means of a cap twister. The yarn obtained had a water imbibition of 90 percent compared with 121.3 percent for an unmodified yarn spun at the same time and under the same conditions.

The bone dry yarn strength of the yarn was 4.70 grams per denier compared with 4.20 grams per denier for the unmodified yarn. The conditioned yarn had a strength of 3.29 grams per denier compared with 2.94 grams per denier for the conditioned unmodified yarn.

The stained cross-sections of the yarns obtained are shown in Figure 2.

Figure 2 shows clearly the "dog-bone" or bean-shaped form of the modified yarn, its non-crenulated surface, thick skin, and diffuse boundary between the skin and core as compared with the unmodified yarn in Figure 1 with its substantially circular cross-section, crenulated surface, thin skin and sharp boundary between the skin and core.

#### Example 2

A viscose was prepared by the method described in Example 1 but was modified by the addition of 1 millimole of triethylene tetramine per 100 grams of viscose. The viscose was spun under similar conditions to those described for Example 1 except that the salt figure was 12.5, the spinning speed was 30 yards per minute and the hot stretch bath contained boiling water and was two feet long. The cross-section of the yarn produced was similar to that shown by Example 1.

#### Example 3

Viscose containing 7.8 percent of cellulose, 6.5 percent of caustic soda and 2.15 percent of combined sulphur was prepared in the usual manner. When the viscose was 33 hours old from the beginning of the mixing stage and the salt figure was 6.5, 0.5 percent of carbon disulphide on the weight of the viscose was added and was mixed in for half an hour at 15° centigrade. 4 millimoles per 100 grams of viscose of diethylene tri-

amine was added and the viscose was mixed for a further half an hour. When the viscose was 45 hours old and had a salt figure of 7.6 it was ready for spinning.

The viscose was extruded through a jet having 40 holes, 0.003 inch in diameter into a coagulating bath containing 9.0 percent of sulphuric acid, 20.0 percent of sodium sulphate and 4.0 percent of zinc sulphate to give a thread of 150 denier and 40 filaments. The length of immersion in the bath was 21 inches and the temperature of the bath was 48° centigrade. The thread was drawn from the bath at a rate of 48.6 metres per minute by a godet and then travelled to a second godet rotating at a higher speed than the first godet, to impart a 20 percent stretch to the thread. The thread was collected in a centrifugal spinning box rotating at 7,000 R. P. M. The cake obtained was washed free from acid and dried.

The distance from the jet at which the freshly coagulated thread became neutral was 8 inches whereas an unmodified viscose extruded under similar conditions became neutral 2 1/4 inches from the jet. The percentage of cellulose in the cake was 40 percent compared with 28.5 percent for an unmodified viscose. The water imbibition of the finished thread was 85 percent compared with 101 percent for a similar thread from an unmodified viscose. Determination of the axial diffusion of the thread was carried out as described by Hermanns in the Textile Research Journal 1948, page 9, using Solophenyl Fast Blue-green BL; no penetration of dyestuff was obtained, but for thread from an unmodified viscose it was 50 $\mu$  after impregnation for four hours in 1 percent solution of the dyestuff at room temperature indicating that the thread from the modified viscose showed no skin and core effect. The thread had a non-crenulated surface and the filaments were dog-bone shape in cross-section.

#### Example 4

Viscose containing 7.8 percent cellulose, 6.5 percent caustic soda and 2.15 percent combined sulphur was prepared in the usual manner and filtered. When the viscose was 16 hours old 0.5 percent of carbon disulphide was added to it and mixed in for 15 minutes. The temperature of the viscose was reduced by cooling to 1° centigrade and divided into four parts to which were added 1.0, 2.0, 3.0 and 6.0 millimoles per 100 grams viscose of triethylene tetramine. The viscoses were mixed for 15 minutes, evacuated for eight hours and spun through a jet having 500 holes, .003 inch in diameter in a bath containing 9.5 percent of sulphuric acid, 20.0 percent of sodium sulphate and 4.0 percent of zinc sulphate at 48° centigrade. The filaments were drawn off by a godet at 18 yards per minute and stretched through a boiling water bath, by means of a second godet having a peripheral speed of 30 yards per minute. The thread was collected in a Topham box revolving at 4,000 R. P. M. The yarn was subsequently washed and dried.

The salt figures of the viscose at the time of spinning were 12.5, 11.4, 11.6 and 10.2 respectively. The stained cross-sections of the yarns are shown in Figures 3, 4, 5 and 6, in which Figure 3 is from viscose having 1.0 millimole of triethylene tetramine per 100 grams of viscose, Figure 4 is from viscose having 2.0 millimoles of triethylene tetramine per 100 grams of viscose, Figure 5 is from viscose having 3 millimoles of triethylene tetramine per 100 grams of viscose and Figure 6 is from viscose having 6.0 millimoles of triethylene tetramine per 100 grams of viscose. These figures show how the shape, smoothness of outline and skin thickness are dependent on the amount of triethylene tetramine present and demonstrate that the optimum concentration for the conditions of the example lies in the region of 1 millimole per 100 grams of viscose.

What we claim is:

1. A process as claimed in claim 3 wherein the poly-  
75 ethylene polyamine is diethylene triamine.

2. A process as claimed in claim 3 wherein the polyethylene polyamine is triethylene tetramine.

3. A process for the production of viscose rayon filaments, threads, fibers and the like having a thick skin comprising extruding viscose, in the presence of more than one quarter of a millimole and less than 5 millimoles per 100 grams of viscose of a polyethylene polyamine component selected from the group consisting of polyethylene polyamines having the general formula



10

where  $n$  is from 1 to 4 inclusive, and condensation products of said polyamines with aliphatic alkylating agents selected from the group consisting of dichlorohydrin, dichlorehylene and trimethylene bromide, into a coagulating bath containing sulphuric acid and 0.5-15% of zinc sulphate.

4. A process for the production of viscose rayon filaments, threads, fibers and the like having a thick skin comprising extruding viscose in the presence of more than one quarter of a millimole and less than 5 millimoles per 100 grams of viscose of a polyethylene polyamine component selected from the group consisting of polyethylene polyamines having the general formula



25

where  $n$  is from 1 to 4 inclusive and condensation products of said polyamines with aliphatic alkylating agents selected from the group consisting of dichlorohydrin, dichlorehylene and trimethylene bromide, into a coagulat-

30

ing bath containing sulphuric acid and 0.5-15% of zinc sulphate, withdrawing the freshly formed thread from the coagulating bath and stretching said thread in a second bath containing hot dilute acid.

5. Viscose containing at least one quarter of a millimole and less than 5 millimoles per 100 grams of viscose of a polyethylene polyamine component selected from the group consisting of polyethylene polyamines of the general formula



where  $n$  is from 1 to 4 inclusive, and condensation products of said polyamines with aliphatic alkylating agents selected from the group consisting of dichlorohydrin, dichlorehylene and trimethylene bromide.

6. Viscose as claimed in claim 5 wherein the polyethylene polyamine is diethylene triamine.

7. Viscose as claimed in claim 5 wherein the polyethylene polyamine is triethylene tetramine.

References Cited in the file of this patent

UNITED STATES PATENTS

|           |              |               |
|-----------|--------------|---------------|
| 1,929,868 | Haller       | Oct. 10, 1933 |
| 2,300,589 | Nelles       | Nov. 3, 1942  |
| 2,312,199 | Tallis       | Feb. 23, 1943 |
| 2,329,086 | Robinson     | Sept. 7, 1943 |
| 2,345,570 | Bley         | Apr. 4, 1944  |
| 2,397,454 | Woodward     | Mar. 26, 1946 |
| 2,422,021 | Kline et al. | June 10, 1947 |
| 2,535,044 | Cox          | Dec. 26, 1950 |